

# United States Patent Office

2,880,087

Patented Mar. 31, 1959

1

2,880,087

## TITANIUM-ALUMINUM ALLOYS

Robert I. Jaffee, Worthington, Ohio, assignor, by mesne assignments, to Crucible Steel Company of America, Flemington, N.J., a corporation of New Jersey

No Drawing. Application January 18, 1957

Serial No. 634,813

13 Claims. (Cl. 75—175.5)

This invention pertains to alloys of titanium and aluminum containing from more than 8% to under 34% aluminum, with and without additions of other alloying elements as specified hereinafter.

This application is a continuation-in-part of copending application Serial No. 401,054, filed December 29, 1953, now abandoned, which is in turn a continuation-in-part of application Serial No. 295,938, filed June 27, 1952, now abandoned, Serial No. 179,322, filed August 14, 1950, now abandoned, and Serial No. 66,838, filed December 22, 1948, and now abandoned, and is also a continuation-in-part of copending application Serial No. 545,121, filed October 24, 1955, which is in turn a continuation-in-part of application Serial No. 392,052, filed November 13, 1953, and now abandoned.

The metal titanium at ordinary temperatures is of a close-packed hexagonal structure commonly called the alpha phase. At a temperature of about 885° C., it is transformed to a body-centered cubic structure known as the beta phase. The addition of aluminum tends to stabilize the alpha phase. Our investigations have established that titanium-aluminum binary alloys containing up to 25% aluminum are found to consist entirely of equiaxed alpha grains. When the aluminum content is increased to about 30% another phase appears interspersed with the alpha phase in a plate-like structure. This additional phase is not beta titanium but a third crystalline form which, due to its high aluminum content, cannot be called a phase of titanium. For the purpose of this specification, it will be identified as I(Al—Ti). Its crystalline form is face-centered tetragonal. When the aluminum content is increased to about 32%, alpha titanium is still present, but at an aluminum content of about 34%, the alpha titanium disappears, and the entire microstructure is one of equiaxed I(Al—Ti) grains. A photomicrograph shows a strong resemblance to many of the brasses. As the aluminum content is further increased, the alloy continues single phase I(Al—Ti) up to an aluminum content of about 46%. At an aluminum content of about 50%, the alloy again has a two-phase microstructure.

In the previously filed applications referred to, we have shown that titanium-aluminum alloys containing 8% and under of aluminum are sufficiently ductile to be hot and cold formed as by forging, rolling, drawing, etc., and that they also possess relatively high strength, particularly in the range of about 2.5 to 8% aluminum. As was further shown in said earlier applications, as the aluminum content is increased above 8%, the binary titanium-aluminum alloys become increasingly brittle, but can be fabricated by hot working up to at least 12% aluminum, and are usable in cast form for higher aluminum contents. It was further shown that these hot workable alloys containing from more than 8% up to at least 12% aluminum have very desirable hot hardness properties.

I have further discovered that the hot workability of titanium-aluminum alloys containing from more than 8% up to about 34% aluminum is greatly improved by additions of one or more of the beta-stabilizing elements Mo, V, Cb, Ta, Mn, Cr, Fe, W, Co, Ni, Cu, Si and Be, and also by additions of certain alpha-stabilizing elements,

2

such as carbon, silver, germanium and zirconium. I have also discovered that such additions greatly increase the strength and ductility of these alloys at both room and elevated temperatures.

5 Carbon is beneficial up to about 0.3% with aluminum up to about 10%; silver, germanium and zirconium are beneficial up to about 5% with aluminum up to at least 10-15%. The lower effective limit for carbon is about 0.05% and for Ag, Ge, and Zr about 0.5%.  
10 Of the beta promoters, those of the beta-isomorphous group Mo, V, Cb and Ta, especially vanadium, are effective up to 40% or more. The eutectoid beta promoters such as Mn, Fe, Co, Ni, Cu, etc., particularly manganese and copper, are effective up to about 10-15% with aluminum up to about 15%. The lower effective limit for the beta promoters is about 0.5%.  
15 Of the interstitials carbon, oxygen and nitrogen, only carbon is a beneficial addition up to about 0.3% as regards improvement in hot workability and strength of the high aluminum, Ti—Al alloys of the invention. Nitrogen and oxygen in amounts of 0.1% each impair hot workability. Of the alpha promoters, silver in amounts up to about 5% is beneficial to hot workability of these alloys, while germanium in amounts up to about 5% is particularly effective in imparting increased hot workability as well as excellent strength and ductility.

20 The following Table I gives the results of tests as to the hot workability in forging and rolling at elevated temperatures of typical alloys according to the invention. In this tabulation, the specimens are rated as follows according to forgeability and rollability at the indicated forging or rolling temperatures, to wit: G=good; F=fair; P=poor; N=G=wholly unfabricable.

35 TABLE I  
Fabrication ratings of Ti—Al and Ti—Al—X alloys containing over 8% Al

| 40               | Composition, Percent (Balance Titanium) | Forging    |        | Rolling    |        | As Cast Hardness, VHN |
|------------------|-----------------------------------------|------------|--------|------------|--------|-----------------------|
|                  |                                         | Temp., °F. | Rating | Temp., °F. | Rating |                       |
| 10Al             |                                         | 1,800      | P      | 1,700      | F-P    |                       |
| 10Al—0.25C       |                                         |            |        | 1,600      | F-G    | 419                   |
| 45 12.5Al—0.25C  |                                         |            |        | 1,800      | N-G    |                       |
| 10Al—2Cu         |                                         | 1,800      | G-F    | 1,700      | N-G    | 286                   |
| 10Al—4Cu         |                                         | 1,800      | G      | 1,700      | G-F    | 412                   |
| 10Al—5Cu         |                                         | 2,000      | G-F    | 1,700      | G      |                       |
| 10Al—6Cu         |                                         | 1,800      | G      | 1,700      | G      | 428                   |
| 12Al—4Cu         |                                         | 1,800      | G      | 1,700      | P      | 418                   |
| 12Al—6Cu         |                                         | 1,800      | G      | 1,700      | G-F    | 466                   |
| 25 12Al—8Cu      |                                         | 1,800      | G      | 1,700      | G      | 446                   |
| 12Al—12Cu        |                                         | 1,800      | F      | 1,700      | F      | 529                   |
| 14Al—4Cu         |                                         | 1,800      | F-P    | 1,700      | N-G    | 414                   |
| 14Al—6Cu         |                                         | 1,800      | F-P    | 1,700      | N-G    | 401                   |
| 15Al—10Cu        |                                         | 1,800      | N-G    | 1,700      | N-G    | 461                   |
| 30Al—5Cu         |                                         | 1,800      | N-G    | 1,700      | N-G    | 341                   |
| 10Al—5Ag         |                                         | 1,800      | P      | 1,700      | P-N-G  | 315                   |
| 10Al—5Ni         |                                         | 1,800      | G      | 1,700      | G      | 465                   |
| 55 10Al—5V       |                                         | 1,800      | G      | 1,700      | G-F    | 390                   |
| 10Al—5Co         |                                         | 1,800      | G      | 1,700      | G      | 498                   |
| 10Al—5Mn         |                                         | 1,800      | G      | 1,700      | G      | 538                   |
| 10Al—5Mo         |                                         | 1,800      | G-F    | 1,700      | G-F    | 432                   |
| 10Al—2.5Fe       |                                         |            |        | 1,800      | G      | 421                   |
| 10Al—5Fe         |                                         |            |        | 1,800      | G      | 363                   |
| 10Al—2.5Ag       |                                         | 1,800      | F      | 1,600      | F      | 317                   |
| 60 10Al—5Ag      |                                         | 1,800      | N-G    |            |        |                       |
| 10Al—2.5Mo—0.25C |                                         |            |        | 1,600      | N-G    |                       |
| 10Al—2.5Ge       |                                         |            |        | 1,800      | G      | 402                   |
| 10Al—2Mn         |                                         |            |        | 1,800      | G      | 402                   |
| 10Al—5Mn         |                                         |            |        | 1,800      | G      | 364                   |
| 10Al—10Mn        |                                         |            |        | 1,800      | G      | 334                   |
| 12.5Al—5Mn       |                                         |            |        | 1,800      | G      | 337                   |
| 12.5Al—10Mn      |                                         |            |        | 1,800      | G      | 403                   |
| 15Al—5Mn         |                                         |            |        | 1,800      | G      | 364                   |
| 65 15Al—10Mn     |                                         |            |        | 1,800      | G      | 442                   |
| 20Al—5Mn         |                                         |            |        | 1,800      | N-G    | 501                   |
| 10Al—2.5Mo       |                                         |            |        | 1,600      | F-P    | 388                   |
| 10Al—0.1N        |                                         |            |        | 1,800      | N-G    |                       |
| 10Al—0.1O        |                                         |            |        | 1,800      | N-G    |                       |
| 10Al—2.5Zr       |                                         |            |        | 1,800      | G      | 384                   |
| 10Al—5Zr         |                                         |            |        | 1,800      | G      | 387                   |
| 70 12.5Al—2.5Zr  |                                         |            |        | 1,800      | N-G    |                       |
| 8.25Al—42.5V     |                                         |            |        | G          | G      |                       |

It will be seen that, whereas the Ti—10Al alloy has only an F-P, i.e., fair-to-poor rating in hot rollability, the addition of 0.25% carbon increases the rating to F-G, i.e., fair-to-good, while the addition of 2.5% zirconium or germanium, or 5% of practically all of the various beta promoters, increases the hot rollability rating to G, i.e., good or excellent. It will further be noted from this data, that although as above stated, the Ti—Al binary alloys cannot be hot worked above about 12% aluminum, at which aluminum level the fabricability is extremely poor, addition of such beta promoters as copper and manganese, impart excellent hot rollability at the 12% aluminum level and even up to 15% thereof.

Although, as above stated, the Ti—Al binary alloys may be hot worked with up to about 12% aluminum, the thus fabricated material has at room temperature no measurable ductility and an extremely low tensile strength of less than 40,000 p.s.i. Additions of various alpha and/or beta promoters aforesaid, in addition to enhancing the hot workability of the binary alloy, also impart greatly enhanced strength and ductility to the resulting hot worked alloy. This is shown by the room temperature mechanical properties given in the following Table II, for representative alloys as fabricated in accordance with Table I and thereafter annealed.

TABLE II

Room temperature mechanical properties of hot workable Ti—Al and Ti—Al—X alloys containing over 8% Al in the condition as rolled and annealed

| Composition, Percent (Balance Titanium) | Tensile Properties, p.s.i. $\times 1,000$ |                   | Percent Elongation in 1" | Percent Reduction in Area | Hardness, VHN |
|-----------------------------------------|-------------------------------------------|-------------------|--------------------------|---------------------------|---------------|
|                                         | 0.2% Offset Yield                         | Ultimate Strength |                          |                           |               |
| 10Al                                    | 40                                        |                   |                          |                           |               |
| 10Al—0.25C                              | 124                                       | 0                 | 1                        | 410                       |               |
| 10Al—2.5Fe <sup>a</sup>                 | 85                                        | 113               | 4                        | 421                       |               |
| 10Al—2Mn                                | 129                                       | 137               | 5                        | 402                       |               |
| 10Al—5Mn                                | 136                                       | 0                 | 0                        | 364                       |               |
| 12.5Al—5Mn                              | 104                                       | 107               | 2                        | 337                       |               |
| 10Al—2.5Mo                              | 166                                       | 178               | 4                        | 388                       |               |
| 8.25Al—46.7V                            | 133                                       | 134               | 10                       | 317                       |               |
| 10Al—2.5Ge <sup>b</sup>                 | 150                                       | 155               | 3                        | 402                       |               |
| 10Al—2.5Ge <sup>c</sup>                 | 112                                       | 114               | 5                        | 348                       |               |
| 10Al—4Cu                                | 103                                       | 0                 | 0                        | 406                       |               |
| 10Al—6Cu                                | 115                                       |                   |                          | 407                       |               |

<sup>a</sup> As quenched from 975° C.

<sup>b</sup> As annealed at 850° C.

<sup>c</sup> As quenched from 950° C.

It will be seen from the data of Table II that the addition of 0.25% carbon greatly increases the strength of the Ti—10Al alloy and also imparts a measurable degree of ductility thereto as shown by the reduction in area value. Also that germanium additions as well as those of the various beta promoters impart excellent tensile strength accompanied in general by good to excellent ductilities, for aluminum contents ranging up to about 12-13%. Thus by virtue of these alloying additions, these extremely weak and brittle binary Ti—Al alloys are converted into strong, ductile and fabricable alloys which, being relatively light in weight by virtue of the high aluminum content, are of great industrial utility, particularly for airplane structural members and certain engine components.

The alloying additions aforesaid also increase the as cast strength of the binary Ti—Al alloys as shown by the data in the following Table III.

TABLE III

Room temperature mechanical properties of Ti—Al and Ti—Al—X alloys containing over 8% Al in the as cast condition

| Composition Percent (Balance Titanium) | Tensile Properties, p.s.i. $\times 1,000$ |                   | Percent Elongation in 1" | Percent Reduction in Area | Hardness, VHN |
|----------------------------------------|-------------------------------------------|-------------------|--------------------------|---------------------------|---------------|
|                                        | 0.2% Offset Yield                         | Ultimate Strength |                          |                           |               |
| 10Al                                   |                                           | 82                | 0                        | 0                         | 309           |
| 15Al                                   |                                           | 10                | 0                        | 0                         | 345           |
| 20Al                                   |                                           | 26                | 0                        | 0                         | 349           |
| 30Al                                   |                                           | 40                | 0                        | 0                         | 431           |
| 36Al                                   |                                           |                   |                          |                           | 256           |
| 15Al—2.5V                              |                                           | 42                | 0                        | 0                         | 364           |
| 30Al—5V                                |                                           | 40                | 0                        | 0                         | 418           |
| 15Al—2.5Cr                             |                                           | 127               | 0                        | 0                         | 418           |
| 15Al—2.5Mo                             |                                           | 110               |                          |                           | 435           |
| 15Al—2.5Fe                             |                                           | 70                | 0                        | 0                         | 374           |
| 15Al—2.5Mn                             |                                           | 60                | 0                        | 0                         | 354           |

As will be seen from the above data, whereas the Ti—15Al binary alloy has an as cast tensile strength of but 10,000 p.s.i. this is increased 40,000 p.s.i. and even up to as much as 130,000 by the beta promoter additions shown.

The beta promoter additions aforesaid also impart excellent elevated temperature tensile properties to these high aluminum-bearing Ti—Al base alloys as shown by the data in the following Table IV.

TABLE IV

Tensile properties at 1000° F. of Ti—(8-12) Al alloys

| Composition, Percent (Balance Titanium) | Tensile Properties, p.s.i. $\times 1,000$ |                   | Percent Elongation in 1" | Percent Reduction in Area |
|-----------------------------------------|-------------------------------------------|-------------------|--------------------------|---------------------------|
|                                         | 0.2% Offset Yield                         | Ultimate Strength |                          |                           |
| 10Al—2Cu                                |                                           | 88                | 125                      |                           |
| 10Al—4Cu                                |                                           | 87                | 126                      | 30                        |
| 10Al—6Cu                                |                                           | 93                | 118                      | 50                        |
| 12Al—8Cu                                |                                           | 64                | 107                      | 5                         |
| 10Al—5Co                                |                                           | 43                | 81                       | 5                         |
| 10Al—5Ni                                |                                           | 59                | 79                       | 15                        |

The alloys of the above table were annealed prior to testing for mechanical properties at 1000° F.

I have found, as above stated, that the binary alloys containing as much as 12% aluminum, can be fabricated by hot working and that these also have very desirable "hot hardness" properties. For example, an alloy containing 12% aluminum, balance substantially all titanium, showed average Vickers hardnesses at various temperatures as shown in the following Table V.

TABLE V

| Temperature, ° C. | Maximum | Vickers Minimum | Hardness Average |
|-------------------|---------|-----------------|------------------|
| 25                |         | 354             | 317              |
| 200               |         | 309             | 287              |
| 300               |         | 287             | 282              |
| 400               |         | 270             | 232              |
| 500               |         | 244             | 230              |
| 600               |         | 236             | 218              |
| 700               |         | 193             | 185              |
| 800               |         | 138             | 133              |

In the test data of Table V, the specimens were hot rolled at 1050° C. to a 28% cross-sectional area reduction, and then annealed for two hours in air at 1000° C. and the surface cleaned and polished prior to hardness testing. The improvement over substantially pure titanium is very marked, the latter having for example, a Vickers hardness of not over 14 at 800° C., as compared to a hardness of at least 130 Vickers for the Ti—12Al alloy at this temperature.

The alloys aforesaid containing beta promoter additions up to about 12 or 14% in general have a mixed alpha-beta microstructure as quenched from the beta field, while those containing upwards of about 15% of total beta promoter content, in general have a substantially all-beta structure as thus quenched. As shown by the Ti-Al-V analyses in the above Table I, the improvement in strength combined with high ductility imparted to these high aluminum, titanium base alloys, is much greater where the beta promoter content is sufficiently high to impart an all-beta structure as quenched, than for lower beta promoter additions imparting a mixed alpha-beta structure.

The alloys of the invention were prepared by arc melting in a cold mold furnace in an inert or argon atmosphere.

What is claimed is:

1. An alloy consisting essentially of: from more than 8 to 15% aluminum, up to 0.3% carbon, about 0.5 to 50% of at least one beta promoting element but not to exceed 15% in total amount of eutectoid beta promoting elements, balance substantially titanium, characterized in being hot workable and in having a minimum tensile strength of about 100,000 p.s.i., as hot worked and annealed.

2. An alloy consisting essentially of: from more than 8 to 15% aluminum, up to 0.3% carbon, about 0.5 to 50% vanadium, balance substantially titanium, characterized in being hot workable and in having a minimum tensile strength of about 100,000 p.s.i. and a minimum tensile elongation of about 2%, as hot worked and annealed.

3. An alloy consisting essentially of: from more than 8% to about 15% aluminum, up to about 0.3% carbon, up to about 50% of beta promoting elements but not to exceed 15% in total amount of eutectoid beta promoting elements, up to about 5% each of silver, and germanium, balance substantially titanium, characterized in being hot workable at about 1800° F.

4. An alloy consisting essentially of: from more than 8% to about 15% aluminum, about 0.5 to 12% copper, balance substantially titanium, characterized in being hot workable at about 1700-1800° F., and in having at 1000° F., a tensile strength of at least 100,000 p.s.i., and a tensile elongation of at least 5%.

5. An alloy consisting essentially of: from more than 8% to about 15% aluminum, about 0.5 to 10% manganese, balance substantially titanium, characterized in being hot workable at about 1800° F., and in having in the hot worked and annealed condition, a tensile strength of at least 100,000 p.s.i. and a tensile elongation of at least 2%.

6. An alloy consisting essentially of: from more than 8% to about 10% aluminum, about 0.5 to 5% germanium, balance substantially titanium, characterized in being hot workable at about 1800° F., and in having a tensile strength of at least 100,000 p.s.i. and a tensile elongation of at least 2%.

7. An alloy consisting essentially of: from more than 8% to about 10% aluminum, about 0.5 to 5% of metal of the group cobalt and nickel, balance substantially titanium, characterized in being hot workable at about 1700-1800° F., and in having a tensile strength at 1000° F. of about 80,000 p.s.i. and a tensile elongation of at least 5%.
8. An alloy consisting essentially of: from more than 8% to about 10% aluminum, about 0.5 to 50% vanadium, balance substantially titanium, characterized in being hot workable at about 1700-1800° F.
9. An alloy consisting essentially of: from more than 8% to about 10% aluminum, about 15 to 50% vanadium, balance substantially titanium, characterized in being hot workable at about 1700-1800° F., and in having a substantially all-beta structure as quenched from the beta field, a tensile strength of at least 100,000 p.s.i. and a tensile elongation of at least 2%, in the hot worked and annealed condition.
10. A cast alloy consisting essentially of: from more than 8% to under 34% aluminum, about 0.5 to 5% of at least one beta promoting element, balance substantially titanium, characterized in having a tensile strength of at least 40,000 p.s.i.
11. An alloy consisting essentially of: from more than 8% to about 12% aluminum, balance substantially titanium, characterized by high hot hardness at temperatures up to about 800° C., and in being hot workable at about 1050° C.
12. An alloy consisting essentially of: from more than 8% to about 10% aluminum, about 0.5 to 5% molybdenum, balance substantially titanium, characterized in being hot workable at about 1700-1800° F.
13. An alloy consisting essentially of: from more than 8% up to 34% aluminum, up to 50% of isomorphous beta promoters for aluminum contents up to 15%, up to 15% of eutectoid beta promoters for aluminum contents up to 15%, up to 5% each of germanium and silver for aluminum contents up to 15%, up to 0.3% carbon, and the balance substantially titanium, characterized by an ultimate strength of at least 40,000 p.s.i.

#### References Cited in the file of this patent

##### UNITED STATES PATENTS

|    |           |               |       |               |
|----|-----------|---------------|-------|---------------|
| 45 | 2,370,289 | Chandler      | ----- | Feb. 27, 1945 |
|    | 2,464,836 | Thomas        | ----- | Mar. 22, 1949 |
|    | 2,550,447 | Blumenthal    | ----- | Apr. 24, 1951 |
|    | 2,554,031 | Jaffee et al. | ----- | May 23, 1951  |
|    | 2,578,098 | Southard      | ----- | Dec. 11, 1951 |
| 50 | 2,596,486 | Jaffee        | ----- | May 13, 1952  |
|    | 2,703,278 | Finlay et al. | ----- | Mar. 1, 1955  |
|    | 2,711,960 | Methe         | ----- | June 28, 1955 |
|    | 2,754,205 | Jaffee et al. | ----- | July 10, 1956 |

##### FOREIGN PATENTS

|         |               |       |                |
|---------|---------------|-------|----------------|
| 681,143 | Germany       | ----- | Sept. 15, 1939 |
| 679,705 | Great Britain | ----- | Sept. 24, 1952 |